

# UNITED STATES PATENT OFFICE.

JOHN FERLÀ, OF NEW YORK, N. Y., ASSIGNOR TO AMERICAN MINERAL WOOD  
MANUFACTURING COMPANY, A CORPORATION OF NEW YORK.

## INSULATING MATERIAL.

1,165,164.

Specification of Letters Patent. Patented Dec. 21, 1915.

No Drawing.

Application filed May 16, 1907. Serial No. 374,044.

*To all whom it may concern:*

Be it known that I, JOHN FERLÀ, a citizen of the Republic of Switzerland, residing in New York city, New York, have invented a 5 new and useful Improvement in Insulating Material, of which the following is a specification.

This invention relates to insulating material and it has for its object the production 10 of an insulating material which can be readily cut and worked with ordinary wood-working tools, which is comparatively inexpensive to produce, and which is adapted for use in insulating conductors for electric currents of high potential.

The invention also contemplates the provision of an insulating material which is thoroughly fire-proof and sufficiently strong to withstand rough handling without danger 20 of breakage.

In producing the improved insulating material, I preferably proceed as follows: I take asbestos and hemp, cut and crush them both into very small and fine pieces by means 25 of special cutting machinery and a revolving crusher, then with these ingredients I mix cement (and coloring matter if desired) in the dry state. For this mixing a rotary machine or revolving kettle is preferably employed. The dry mixture of asbestos, hemp, 30 cement and coloring matter is then transferred to another mixer where acetic acid, liquid glue and water are added. The quantity of water added at this stage is sufficient 35 to moisten the ingredients thoroughly and form a moderately thick paste. The mixture is then transferred to a large tank provided with an agitator to prevent the solid material from settling or becoming hardened 40 and from this tank the pasty mass is transferred to a canal where an excess of water is added to make the material flow freely. The highly fluid mixture is flowed from the canal upon a moving or revolving web, such 45 as wire cloth of suitable mesh, in order to allow the excess water to drain out of the material. After the water has been allowed to drain off for a time the material is passed onto a strip of felt or like material and is 50 subjected to light pressure, preferably through the agency of rollers, which gage the thickness of the sheet of material and also express some of the residual water, which is absorbed by the felt. After the

material is hardened enough to be handled 55 with safety, it is cut into sheets of the desired dimensions and these are subjected to heavy pressure in a powerful press, the pressing operation being preferably carried on in a pressure chamber from which the 60 air is exhausted in order to facilitate the removal of the water still remaining in the material. After being subjected to pressure a sufficient length of time, the material is allowed to dry and is then preferably heated 65 to a temperature of five or six hundred degrees, and placed in a bath of linseed oil, which may be either raw or boiled. After having been allowed to stand for a sufficient length of time in the bath of oil, the material is removed and baked in an oven to 70 effect the rapid drying of the oil. The addition of the acetic acid to the mixture prevents the composition from becoming hard and brittle with age, and tends to maintain 75 its easily workable characteristics. The acetic acid seems to prevent a kind of petrification to which mixtures of asbestos and cement are subject after any considerable period of time. The asbestos and hemp 80 fibers form the body of the compound and cement forms a sort of filling medium which occupies the spaces among the fibers. It is true that the cement when mixed also serves to some extent as a binder, but this function 85 is mainly performed by the glue and the acid produces a suitable degree of hardness. The resulting material is characterized by a high degree of electrical non-conductivity, is fire-proof, considerably harder than the wood, 90 and yet is adapted to be handled and worked with the tools ordinarily employed in wood-working.

While I preferably employ asbestos, hemp, cement, acetic acid and glue in preparing the 95 material which is subjected to the treatment with oil, the characteristic qualities of my material may be obtained in a measure by the use of asbestos and cement alone in the preparation of the material to be treated 100 with the oil. The material so produced has not the same degree of toughness as when all of the materials above mentioned are employed, and I therefore preferably make use of the additional materials already mentioned; but I do not wish to be understood as limiting myself to a compound comprising 105 all of the ingredients enumerated.

While it is desirable to heat the asbestos and cement composition before introducing it into the oil and such a preliminary heating increases the effectiveness of the treatment with oil, the composition may be introduced into the oil without preliminary heating and the resulting material is characterized by the same properties as that produced when the composition is first heated before introduction into the oil, but the insulating properties are not present in such high degree.

While I have mentioned only linseed as suitable for use in making the insulating material, it is to be understood that other oils of similar properties may be employed instead, and it is probable that other drying oils will give satisfactory results. It is also obvious that other binding materials than those which I have mentioned may be used with the asbestos to form the composition which is soaked in oil, and I do not limit myself to the employment of the binding materials specified, though those binding materials give the best results which I have obtained.

Having thus described my invention, what I claim is new and desire by Letters Patent is:

1. The composition of matter comprising, a mixture of cement, hemp, mineral fiber,

acetic acid and glue, impregnated with a drying oil.

2. The process of forming a composition of matter which comprises mixing cement and fibrous material, then adding a liquid gelatinous binder and water to form a liquid paste, removing the surplus water, impregnating with a drying oil, and then drying or oxidizing said oil.

3. The process of forming a composition of matter which comprises, mixing cement, hemp and asbestos, then adding water, acetic acid and glue to form a liquid paste, removing the surplus liquid, impregnating with a drying oil, and then drying or oxidizing said oil.

4. A composition of matter comprising a medium forming a body, a filler and binder, an agent for preventing undue hardening, and a drying oil.

5. A composition of matter comprising a medium forming a body, a filler, a binder, an agent for preventing undue hardening, and a drying oil.

In testimony whereof, I have signed my name in the presence of two witnesses.

JOHN FERLA.

Witnesses:

J. FRANK GUIMARAEZ,  
WM. BRADFORD.